# EUROPEAN PATENT APPLICATION

(11) **EP 4 779 047 A1**
(43) Date of publication of application: **22.07.2026**
(21) Application number: 24888287.0
(22) Date of filing: 02.07.2024
(51) Int. Cl.: C22C 38/00, B21C 37/08, C21D 8/10, C22C 38/38, C22C 38/58

(54) **ELECTRIC-RESISTANCE-WELDED STEEL PIPE, LINE PIPE, AND METHOD FOR PRODUCING ELECTRIC-RESISTANCE-WELDED STEEL PIPE**

(30) Priority: 09.11.2023 JP 2023191290
(71) Applicant: JFE Steel Corporation, Tokyo 100-0011 (JP)
(72) Inventor: MATSUMOTO Akihide, Tokyo 100-0011 (JP); IWATA Naomichi, Tokyo 100-0011 (JP); EGUCHI Kenichiro, Tokyo 100-0011 (JP)
(74) Representative: Haseltine Lake Kempner LLP
(86) International application number: PCT/JP2024/023975
(87) International publication number: WO 2025/099985

(57) **Abstract**

In an aspect, an electric resistance welded steel pipe with excellent corrosion resistance is provided. The electric resistance welded steel pipe includes a base metal material, and an electric resistance weld connecting one end portion of the base metal material and other end portion of the base metal material to each other. The base metal material and the electric resistance weld of the electric resistance welded steel pipe contain at least one of Cr, Mo, or Cu. Relationships between the concentrations of Cr, Mo, and Cu in the base metal material and the concentrations of Cr, Mo, and Cu in the electric resistance weld satisfy predetermined expressions. The electric resistance welded steel pipe and other aspects provided according to the present invention can realize excellent corrosion resistance.

## Description

### Technical Field

The present invention relates to an electric resistance welded steel pipe suitably used as a line pipe in a pipeline, to a line pipe, and to a method for manufacturing an electric resistance welded steel pipe.

### Background Art

In recent years, carbon dioxide capture and storage (CCS) has attracted attention as a global warming countermeasure. In this technology, CO₂ that will be emitted into the air is captured and stored underground. The CCS mainly captures CO₂ generated in industrial facilities, such as power plants and factories. The captured CO₂ is transported to storage sites via pipelines. This CO₂ contains SOₓ and NOₓ that are generated from the combustion of coals or natural gases. These gases, when dissolved in water, form strongly acidic sulfuric acid and nitric acid. Thus, pipelines that transport CO₂ emitted from industrial facilities are exposed to a severe corrosive environment.

Efforts have been made to enhance the corrosion resistance of steel materials and steel pipes used as line pipes for such pipelines. For example, Patent Literatures 1 and 2 disclose that such elements as Cr and Cu are added to steel sheets or the like.

### Citation List

### Patent Literature

PTL 1: Japanese Unexamined Patent Application Publication No. 2000-199029
PTL 2: Japanese Patent No. 4499949

### Summary of Invention

### Technical Problem

Here, an example of the steel pipes used as line pipes is electric resistance welded steel pipes in which one end side and the other end side of a base metal are connected to each other by electric resistance welding. In the electric resistance welded steel pipe, the electric resistance weld that connects the end portions of the base metal material to each other tends to be poor in corrosion resistance as compared with the base metal material. Thus, even electric resistance welded steel pipes manufactured using the steel materials described in Patent Literatures 1 and 2 still have room for improvement in the corrosion resistance of the electric resistance weld.

The present invention has been made in light of the problems discussed above. It is therefore an object of the present invention to provide, in an aspect, an electric resistance welded steel pipe with excellent corrosion resistance.

### Solution to Problem

In order to solve the above problems, the present invention has the following features.
[1] An electric resistance welded steel pipe including a base metal material, and an electric resistance weld connecting one end portion of the base metal material and other end portion of the base metal material to each other, wherein
   the base metal material and the electric resistance weld contain at least one of Cr, Cu, or Mo, and
   relationships between the concentrations of Cr, Cu, and Mo in the base metal material and the concentrations of Cr, Cu, and Mo in the electric resistance weld satisfy the following expression: ${\left[Cr\right]}_{B} + {\left[Cu\right]}_{B} + {\left[Mo\right]}_{B} \geq 0.02$
   and further satisfy expression (1) when the base metal material contains 0.02 mass% or more Cr; satisfy expression (2) when the base metal material contains 0.02 mass% or more Cu; and satisfy expression (3) when the base metal material contains 0.02 mass% or more Mo, ${\left[Cr\right]}_{W} / {\left[Cr\right]}_{B} \leq 1.50$ ${\left[Cu\right]}_{W} / {\left[Cu\right]}_{B} \leq 1.50$ ${\left[Mo\right]}_{W} / {\left[Mo\right]}_{B} \leq 1.50$
   wherein [Cr]_{B} is the concentration (mass%) of Cr in the base metal material, [Cr]_{W} is the concentration (mass%) of Cr in the electric resistance weld, [Cu]_{B} is the concentration (mass%) of Cu in the base metal material, [Cu]_{W} is the concentration (mass%) of Cu in the electric resistance weld, [Mo]_{B} is the concentration (mass%) of Mo in the base metal material, and [Mo]_{W} is the concentration (mass%) of Mo in the electric resistance weld.
[2] The electric resistance welded steel pipe according to [1], wherein the base metal material has a chemical composition including, in mass%:
   C: 0.020% or more and 0.200% or less,
   Si: 0.50% or less,
   Mn: 0.50% or more and 2.00% or less,
   P: 0.050% or less,
   S: 0.0200% or less,
   Al: 0.005% or more and 0.100% or less, and
   N: 0.0100% or less,
   and further including at least one of:
      Cr: 5.00% or less,
      Cu: 2.00% or less, or
      Mo: 2.00% or less,
      the balance being Fe and incidental impurities.
[3] The electric resistance welded steel pipe according to [2], wherein the chemical composition of the base metal material further includes, in mass%, at least one selected from:
   Nb: 0.080% or less,
   V: 0.080% or less,
   Ti: 0.080% or less,
   Ni: 2.00% or less,
   Ca: 0.0050% or less,
   B: 0.0050% or less, and
   Sn: 0.100% or less.
[4] The electric resistance welded steel pipe according to any one of [1] to [3], which has a difference in Vickers hardness of 100 HV or less in absolute value between the Vickers hardness at a position 1 mm deep from an inner surface of the electric resistance weld and the Vickers hardness at a position 1 mm deep from an inner surface of the base metal material.
[5] A line pipe using the electric resistance welded steel pipe described in any one of [1] to [4].
[6] A method for manufacturing an electric resistance welded steel pipe including a hot-rolled steel sheet producing step of heating and hot-rolling a steel material to produce a hot-rolled steel sheet; a pipe forming step of forming the hot-rolled steel sheet into an open pipe; and a welding step of welding one end portion and other end portion of the open pipe with each other by electric resistance welding, wherein
   the steel material that is heated and hot-rolled to produce a hot-rolled steel sheet in the hot-rolled steel sheet producing step contains Cu, Cr, and Mo in a total amount of 0.02 mass% or more, and
   the welding step is performed under conditions where a temperature of 1000°C or above is reached in 1.0 second or less in central regions in a thickness direction of portions of the open pipe that are to be welded, the portions of the open pipe that are to be welded have an oxygen concentration of 0.10 mass% or less, and the amount of molten steel discharge is 0.2 times or more a sheet thickness of the open pipe.

### Advantageous Effects of Invention

According to the electric resistance welded steel pipe and other aspects of the present invention, the base metal material and the electric resistance weld contain at least one of Cr, Cu, or Mo. Furthermore, the concentrations of Cr, Cu, and Mo in the base metal material and the concentrations of Cr, Cu, and Mo in the electric resistance weld satisfy the predetermined relationships. These configurations can realize excellent corrosion resistance in the electric resistance welded steel pipe and the other aspects.

### Brief Description of Drawings

[Fig. 1] Fig. 1 is an explanatory view illustrating an embodiment of a cross section of an electric resistance welded steel pipe.
[Fig. 2] Fig. 2 is a flow diagram illustrating a method for manufacturing an electric resistance welded steel pipe.
[Fig. 3] Fig. 3 is an explanatory view illustrating an embodiment of the welding step in Fig. 2.

### Description of Embodiments

Hereinbelow, embodiments of the present invention will be described based on the drawings. Fig. 1 illustrates a cross section perpendicular to the axial direction of an electric resistance welded steel pipe 100. The electric resistance welded steel pipe 100 includes a base metal material 10, and an electric resistance weld 20 that connects one end portion 11 of the base metal material 10 and the other end portion 12 of the base metal material 10 to each other. In the present embodiment, the electric resistance welded steel pipe 100 is formed with a cylindrical shape but is not particularly limited thereto.

The base metal material 10 has a C-shaped cross section perpendicular to the axial direction of the electric resistance welded steel pipe 100. The electric resistance weld 20 is a portion formed by thermally melting the base metal material 10, and is also called a bead. The electric resistance weld 20 is disposed between the side having one end portion 11 and the side having other end portion 12 of the base metal material 10 in the circumferential direction of the electric resistance welded steel pipe 100. Heat-affected zones 30 are disposed between the base metal material 10 and the electric resistance weld 20 in the circumferential direction.

The base metal material 10 and the electric resistance weld 20 contain at least one of Cr, Cu, or Mo. In other words, as long as the base metal material 10 and the electric resistance weld 20 have one of these three components, the contents of the other components may be "0 mass%". Here, the concentration (mass%) of Cr in the base metal material 10 is expressed as [Cr]_{B}, and the concentration (mass%) of Cr in the electric resistance weld 20 is written as [Cr]_{W}. The concentration (mass%) of Cu in the base metal material 10 is expressed as [Cu]_{B}, and the concentration (mass%) of Cu in the electric resistance weld 20 is written as [Cu]_{W}. The concentration (mass%) of Mo in the base metal material 10 is expressed as [Mo]_{B}, and the concentration (mass%) of Mo in the electric resistance weld 20 is written as [Mo]_{W}.

Relationships between the concentrations (mass%) of Cr, Cu, and Mo in the base metal material 10 and the concentrations (mass%) of Cr, Cu, and Mo in the electric resistance weld 20 satisfy the following expression. Hereinafter, the "mass%" for the concentrations of Cr, Cu, and Mo will be simply written as "%". ${\left[Cr\right]}_{B} + {\left[Cu\right]}_{B} + {\left[Mo\right]}_{B} \geq 0.02$

The relationships further satisfy expression (1) when the base metal material 10 contains 0.02 mass% or more Cr; satisfy expression (2) when the base metal material 10 contains 0.02 mass% or more Cu; and satisfy expression (3) when the base metal material 10 contains 0.02 mass% or more Mo. ${\left[Cr\right]}_{W} / {\left[Cr\right]}_{B} \leq 1.50$ ${\left[Cu\right]}_{W} / {\left[Cu\right]}_{B} \leq 1.50$ ${\left[Mo\right]}_{W} / {\left[Mo\right]}_{B} \leq 1.50$

The sum of the concentrations of Cr, Mo, and Cu in the base metal material 10 is preferably 0.05% or more, and more preferably 0.10% or more. When the sum of the concentrations of Cr, Mo, and Cu is more than 7.00%, the ductility and the toughness of the electric resistance weld 20 are lowered to facilitate the occurrence of cracking in the electric resistance weld 20. Thus, the sum of the concentrations of Cr, Mo, and Cu in the base metal material 10 is preferably 7.00% or less, and more preferably 6.00% or less.

Chromium is easily oxidized in the air at high temperatures. Thus, Cr oxide is present in the electric resistance weld 20. The surrounding of Cr oxide has a lower Cr concentration and thus has low corrosion resistance.

Here, the "corrosion resistance" can be evaluated based on the corrosion rate and the pitting corrosion growth rate in a corrosion test described later. The corrosion resistance is evaluated as sufficient, good, or the like when the corrosion rate in the corrosion test is, for example, 0.100 mm/year or less and the pitting corrosion growth rate is 0.100 mm/year or less.

When Cr oxide remains in the electric resistance weld 20, the Cr concentration in the electric resistance weld 20 is higher than that in the base metal material 10. The Cr concentration in the regions excluding the Cr oxide is lowered, leading to a decrease in the corrosion resistance of the electric resistance weld 20.

When the base metal material 10 contains 0.02% or more Cr, the Cr concentration in the electric resistance weld 20 relative to that in the base metal material 10, namely, [Cr]_{W}/[Cr]_{B}, is 1.50 or less. By virtue of [Cr]_{W}/[Cr]_{B} being 1.50 or less, the corrosion resistance in the electric resistance weld 20 can be ensured. The ratio [Cr]_{W}/[Cr]_{B} is preferably 1.40 or less, and more preferably 1.30 or less.

When the Cr concentration in the electric resistance weld 20 is excessively lower than that in the base metal material 10, the corrosion resistance of the electric resistance weld 20 may be lowered. In the electric resistance welded steel pipe 100, [Cr]_{W}/[Cr]_{B} is preferably 0.50 or more. The ratio [Cr]_{W}/[Cr]_{B} is more preferably 0.60 or more, and even more preferably 0.70 or more.

Copper is less susceptible to oxidation at high temperatures than Fe. Thus, iron is oxidized preferentially in the electric resistance weld 20, and copper increases its concentration. When concentrated copper remains in the electric resistance weld 20, the Cu concentration in the electric resistance weld 20 is higher than that in the base metal material 10. The difference in Cu concentration between the base metal material 10 and the electric resistance weld 20 forms local cells, which may reduce the corrosion resistance of the heat-affected zones 30.

When the base metal material 10 contains 0.02% or more Cu, the Cu concentration in the electric resistance weld 20 relative to that in the base metal material 10, namely, [Cu]_{W}/[Cu]_{B}, is 1.50 or less. By virtue of [Cu]_{W}/[Cu]_{B} being 1.50 or less, the corrosion resistance in the electric resistance weld 20 can be ensured.

The ratio [Cu]_{W}/[Cu]_{B} is preferably 1.40 or less, and more preferably 1.30 or less. When the Cu concentration in the electric resistance weld 20 is excessively lower than that in the base metal material 10, the corrosion resistance of the electric resistance weld 20 may be lowered. The ratio [Cu]_{W}/[Cu]_{B} is preferably 0.50 or more, more preferably 0.60 or more, and even more preferably 0.70 or more.

Molybdenum is an element that enhances the corrosion resistance of steel. Sufficient corrosion resistance can be obtained in the base metal material 10 by controlling the total concentration of Cr, Cu, and Mo in the base metal material 10 to 0.02% or more.

When the base metal material 10 contains 0.02% or more Mo, [Mo]_{w}/[Mo]_{B} is 1.50 or less. It is recommended that the ratio be 1.40 or less, preferably 1.30 or less. It is recommended that [Mo]_{w}/[Mo]_{B} be 0.50 or more. The ratio [Mo]_{w}/[Mo]_{B} is preferably 0.60 or more, and more preferably 0.70 or more.

The corrosion resistance of the heat-affected zones 30 can be ensured by controlling [Mo]_{w}/[Mo]_{B} to 1.50 or less. The reason for this is specifically described below. Molybdenum in steel is less susceptible to oxidation at high temperatures than Fe. Thus, iron is oxidized preferentially in the electric resistance weld 20, and molybdenum increases its concentration. When concentrated molybdenum remains in the electric resistance weld 20, the Mo concentration in the electric resistance weld 20 is higher than that in the base metal material 10. In such a state, the difference in Mo concentration between the base metal material 10 and the electric resistance weld 20 forms local cells, which may reduce the corrosion resistance of the heat-affected zones 30. The corrosion resistance of the electric resistance weld 20 can be further enhanced by controlling [Mo]_{w}/[Mo]_{B} to 0.50 or more.

[Cr]_{W}, [Cr]_{B}, [Cu]_{W}, [Cu]_{B}, [Mo]_{w}, and [Mo]_{B} may be measured by an EPMA (electron probe micro analyzer) method. The concentrations in the base metal material 10 and in the electric resistance weld 20 may be measured with respect to a measurement surface that is a cross section perpendicular to the axial direction of the electric resistance welded steel pipe 100. In the measurement by the EPMA method, the beam diameter may be set to 1 µm.

Here, the concentrations of the components in the base metal material 10 are measured with respect to a position 90 degrees away from the electric resistance weld 20 in a circumferential direction. The concentrations of the components in the electric resistance weld 20 are measured with respect to the center of the electric resistance weld 20.

More specifically, [Cr]_{B}, [Cu]_{B}, and [Mo]_{B} may be determined by measuring the respective concentrations with respect to a total of 9 sites that are centered at a position 90 degrees away from the electric resistance weld 20 in a circumferential direction and are located 1 mm deep from the inner surface at 1 µm intervals in the circumferential direction, and averaging the measured values.

[Cr]_{W}, [Cu]_{W}, and [Mo]_{w} may be determined by measuring the respective concentrations with respect to a total of 9 sites that are centered at the electric resistance weld 20 and are located 1 mm deep from the inner surface at 1 µm intervals in a circumferential direction, and averaging the measured values.

The base metal material 10 preferably has a chemical composition including, in mass%:
C: 0.020% or more and 0.200% or less,
Si: 0.50% or less,
Mn: 0.50% or more and 2.00% or less,
P: 0.050% or less,
S: 0.0200% or less,
Al: 0.005% or more and 0.100% or less, and
N: 0.0100% or less,
and further including at least one of:
   Cr: 5.00% or less,
   Cu: 2.00% or less, or
   Mo: 2.00% or less,
   the balance being Fe and incidental impurities. In the present specification, "%" indicating the steel chemical composition is "mass%" unless otherwise specified.

### C: 0.020% or more and 0.200% or less

Carbon is an element that increases the strength of steel through solid solution strengthening. Carbon is also an element that lowers the transformation start temperature and thereby reduces the grain size, thus increasing the strength of steel. The base metal material 10 can benefit from these effects by containing 0.020% or more C.

When the base metal material 10 contains an excessively large amount of carbon, hard microstructures are excessively formed in the electric resistance weld 20. As a result, the electric resistance weld 20 is increased in hardness, and the ductility and the toughness of the electric resistance weld 20 are lowered. Furthermore, local cells are formed due to the difference in material properties between the base metal material 10 and the electric resistance weld 20, and may cause a decrease in the corrosion resistance of the heat-affected zones 30.

It is recommended that the C content in the base metal material 10 be 0.200% or less. The C content is preferably 0.180% or less, and more preferably 0.170% or less. It is recommended that the C content in the base metal material 10 be 0.020% or more. The C content is preferably 0.025% or more, and more preferably 0.030% or more. The C content in the base metal material 10 is preferably 0.025% or more and 0.180% or less, and more preferably 0.030% or more and 0.170% or less.

### Si: 0.50% or less

Silicon is an element that increases the strength of steel through solid solution strengthening. The base metal material 10 can benefit from this effect by containing 0.02% or more Si. When the base metal material 10 contains an excessively large amount of silicon, the hardness of the electric resistance weld 20 is increased. As a result, the ductility and the toughness of the electric resistance weld 20 are lowered. Furthermore, local cells are formed due to the difference in material properties between the base metal material 10 and the electric resistance weld 20, and may cause a decrease in the corrosion resistance of the heat-affected zones 30.

It is recommended that the base metal material 10 contain 0.50% or less Si. The Si content is preferably 0.40% or less, and more preferably 0.30% or less. The base metal material 10 preferably contains 0.05% or more and 0.40% or less Si, and more preferably 0.08% or more and 0.30% or less Si.

### Mn: 0.50% or more and 2.00% or less

Manganese is an element that increases the strength of steel through solid solution strengthening. Manganese is also an element that lowers the transformation start temperature and thereby reduces the grain size, thus increasing the strength of steel. The base metal material 10 can benefit from these effects by containing 0.50% or more Mn.

When the base metal material 10 contains an excessively large amount of manganese, hard microstructures are excessively formed in the electric resistance weld 20. As a result, the electric resistance weld 20 is increased in hardness, and the ductility and the toughness of the electric resistance weld 20 are lowered. Furthermore, local cells are formed due to the difference in material properties between the base metal material 10 and the electric resistance weld 20, and may cause a decrease in the corrosion resistance of the heat-affected zones 30.

The base metal material 10 preferably contains 0.05% or more Mn, more preferably 0.60% or more Mn, and even more preferably 0.70% or more Mn. The base metal material 10 preferably contains 2.00% or less Mn, more preferably 1.90% or less Mn, and even more preferably 1.80% or less Mn. The base metal material 10 preferably contains 2.00% or less Mn, more preferably 0.60% or more and 1.90% or less Mn, and even more preferably 0.70% or more and 1.80% or less Mn.

### P: 0.050% or less

Phosphorus is an element that reduces toughness through segregation at grain boundaries. Phosphorus corresponds to an incidental impurity. It is recommended that the base metal material 10 have the lowest content possible of phosphorus. The P content is preferably 0.050% or less, more preferably 0.040% or less, and even more preferably 0.030% or less. The lower limit of the P content is not particularly specified, but excessive dephosphorization increases the smelting costs. Thus, the P content is preferably 0.001% or more.

### S: 0.0200% or less

Sulfur is usually present in steel as MnS. The steel material before the formation of the base metal material 10 is thinly stretched in the hot rolling process. MnS adversely affects the ductility and the toughness of the steel material in the hot rolling process.

The base metal material 10 preferably has the lowest content possible of sulfur. It is recommended that the S content in the base metal material 10 be 0.0200% or less. The S content is preferably 0.0100% or less, and more preferably 0.0050% or less. The lower limit of the S content is not particularly specified, but excessive desulfurization increases the smelting costs. Thus, the S content is preferably 0.0001% or more.

### Al: 0.005% or more and 0.100% or less

Aluminum is an element that acts as a powerful deoxidizing agent. The base metal material 10 can benefit from this effect by containing 0.005% or more Al. When the base metal material 10 contains an excessively large amount of aluminum, weldability is deteriorated and the number of alumina inclusions is increased to cause deterioration in the surface properties of the base metal material 10.

It is recommended that the base metal material 10 contain 0.100% or less Al. The Al content is preferably 0.080% or less, and more preferably 0.070% or less. The base metal material 10 preferably contains 0.010% or more and 0.080% or less Al, and more preferably 0.015% or more and 0.070% or less Al.

### N: 0.0100% or less

Nitrogen is an incidental impurity and is an element that strongly locks dislocation motion, thereby lowering the ductility and the toughness of the base metal material 10. The base metal material 10 preferably has the lowest content possible of nitrogen. Up to 0.0100% N is acceptable. It is recommended that the N content in the base metal material 10 be 0.0100% or less. The N content is preferably 0.0080% or less, and more preferably 0.0060% or less.

### Cr: 5.00% or less

Chromium is an element that enhances corrosion resistance. Furthermore, chromium is an element that contributes to reducing the size of microstructures by lowering the transformation start temperature, and thereby increases the strength of steel. The base metal material 10 can benefit from these effects by containing 0.01% or more Cr. An excessively large amount of chromium leads to deterioration in the ductility and the toughness of the base metal material 10.

When the base metal material 10 contains an excessively large amount of chromium, the hardness of the electric resistance weld 20 may be increased and the corrosion resistance of the heat-affected zones 30 may be lowered. When the base metal material 10 contains an excessively large amount of chromium, a large amount of Cr oxide is formed in the electric resistance weld 20 and the corrosion resistance of the electric resistance weld 20 may be lowered.

It is recommended that the base metal material 10 contain 5.00% or less Cr. The Cr content is more preferably 3.00% or less, and even more preferably 2.00% or less. The base metal material 10 preferably contains 0.02% or more Cr, and more preferably 0.05% or more Cr. The base metal material 10 preferably contains 0.05% or more and 2.00% or less Cr.

### Cu: 2.00% or less

Copper is an element that enhances corrosion resistance. Furthermore, copper is an element that increases the strength of steel through solid solution strengthening. Furthermore, copper is an element that contributes to reducing the size of microstructures by lowering the transformation start temperature, and thereby increases the strength of steel.

The base metal material 10 can benefit from these effects by containing 0.01% or more Cu. When the base metal material 10 contains an excessively large amount of copper, ductility and toughness are lowered. Furthermore, when the base metal material 10 contains an excessively large amount of copper, the hardness of the electric resistance weld 20 may be increased and the corrosion resistance of the heat-affected zones 30 may be lowered. Furthermore, adding copper to the base metal material 10 in an amount exceeding the solid solubility limit results in the occurrence of Cu precipitates and does not increase the amount of copper dissolved in the steel. Thus, such addition does not produce corresponding effects in enhancing corrosion resistance. It is recommended that the base metal material 10 contain 2.00% or less Cu. The Cu content is preferably 1.80% or less, and more preferably 1.60% or less. The base metal material 10 preferably contains 0.02% or more Cu, and more preferably 0.05% or more Cu. The base metal material 10 preferably contains 0.02% or more and 1.80% or less Cu, and more preferably 0.05% or more and 1.60% or less Cu.

### Mo: 2.00% or less

Molybdenum is an element that contributes to reducing the size of microstructures by lowering the transformation start temperature, and thereby increases the strength of steel. The base metal material 10 can benefit from these effects by containing 0.01% or more Mo. When the base metal material 10 contains an excessively large amount of molybdenum, ductility and toughness are lowered. Furthermore, when the base metal material 10 contains an excessively large amount of molybdenum, the hardness of the electric resistance weld 20 may be increased and the corrosion resistance of the heat-affected zones 30 may be lowered. It is recommended that the base metal material 10 contain 2.00% or less Mo. The Mo content is preferably 1.80% or less, and more preferably 1.60% or less. The base metal material 10 preferably contains 0.02% or more Mo, and more preferably 0.05% or more Mo. The base metal material 10 preferably contains 0.02% or more and 1.80% or less Mo, and more preferably 0.05% or more and 1.60% or less Mo.

The base metal material 10 contains Fe and incidental impurities as the balance. Here, the electric resistance welded steel pipe according to an embodiment of the present invention may exclusively contain the components described above and the balance, with the balance being Fe and incidental impurities. Incidental impurities are impurities that are incidentally mixed in from raw materials or via the manufacturing processes, the manufacturing equipment, etc., and may be contained without impairing the object of the present invention. Examples of the raw materials include iron ores, reduced iron, and scrap. Examples of the incidental impurities in the balance include Mg, Zr, REM, Sn, As, Sb, Bi, Co, Pb, Zn, O, Ta, W, Te, Hf, Ge, Sr, and Cs. Here, REM is a general term for a total of 17 elements including Sc, Y, and the lanthanoid elements. The base metal material 10 may contain at least one of these 17 elements as an incidental impurity. The REM content in the base metal material 10 is the total content of these elements.

The chemical composition of the base metal material 10 may further include, in mass%, at least one selected from:
Nb: 0.080% or less,
V: 0.080% or less,
Ti: 0.080% or less,
Ni: 2.00% or less,
Ca: 0.0050% or less,
B: 0.0050% or less, or
Sn: 0.100% or less. Incidentally, Nb, V, Ni, Ca, B, and Sn are elements that may be optionally contained in the base metal material 10. That is, the contents of these components in the base metal material 10 may be "0 mass%".

### Nb: 0.080% or less

Niobium contributes to enhancing the strength of steel by forming fine carbides and nitrides in the steel. Furthermore, niobium is an element that suppresses the coarsening of microstructures during hot rolling and thereby contributes to reducing the size of microstructures, thus increasing the strength of steel.

The base metal material 10 can benefit from these effects by containing 0.002% or more Nb. When the base metal material 10 contains an excessively large amount of niobium, ductility and toughness are lowered.

It is recommended that the base metal material 10 contain 0.080% or less Nb. The Nb content is preferably 0.070% or less, and more preferably 0.060% or less. The base metal material 10 preferably contains 0.005% or more Nb, and more preferably 0.010% or more Nb. The base metal material 10 preferably contains 0.005% or more and 0.070% or less Nb, and more preferably 0.010% or more and 0.060% or less Nb.

### V: 0.080% or less

Vanadium is an element that contributes to enhancing the strength of steel by forming fine carbides and nitrides in the steel. The base metal material 10 can benefit from this effect by containing 0.002% or more V.

When the base metal material 10 contains an excessively large amount of vanadium, ductility and toughness are lowered. It is recommended that the base metal material 10 contain 0.080% or less V. The V content is preferably 0.070% or less, and preferably 0.060% or less. The base metal material 10 preferably contains 0.005% or more V, and preferably 0.010% or more V. The base metal material 10 preferably contains 0.005% or more and 0.070% or less V, and preferably 0.010% or more and 0.060% or less V.

### Ti: 0.080% or less

Titanium is an element that contributes to enhancing the strength of steel by forming fine carbides and nitrides in the steel. Furthermore, titanium is an element that has high affinity for nitrogen and thus contributes to reducing the amount of dissolved nitrogen in steel. The base metal material 10 preferably contains 0.002% or more Ti.

When the base metal material 10 contains an excessively large amount of titanium, ductility and toughness are lowered. When the base metal material 10 contains Ti, it is recommended that the Ti content be 0.080% or less. The Ti content is preferably 0.070% or less, and more preferably 0.060% or less. The base metal material 10 preferably contains 0.005% or more Ti, and more preferably 0.010% or more Ti. The base metal material 10 preferably contains 0.005% or more and 0.070% or less Ti, and more preferably 0.010% or more and 0.060% or less Ti.

### Ni: 2.00% or less

Nickel is an element that increases the strength of steel through solid solution strengthening. Nickel is an element that also contributes to reducing the size of microstructures by lowering the transformation start temperature, and thereby increases the strength of steel. The base metal material 10 can benefit from these effects by containing 0.01% or more Ni. When the base metal material 10 contains an excessively large amount of nickel, ductility and toughness are lowered. Furthermore, when the base metal material 10 contains an excessively large amount of nickel, the hardness of the electric resistance weld 20 may be increased and the corrosion resistance of the heat-affected zones 30 may be lowered. It is recommended that the base metal material 10 contain 2.00% or less Ni. The Ni content is preferably 1.80 or less, and more preferably 1.60% or less. The base metal material 10 preferably contains 0.02% or more Ni, and more preferably 0.05% or more Ni. The base metal material 10 preferably contains 0.02% or more and 1.80 or less Ni, and more preferably 0.05% or more and 1.60% or less Ni.

### Ca: 0.0050% or less

Calcium is an element that contributes to enhancing the toughness of steel by spheroidizing sulfides, such as MnS, that are thinly elongated in the hot rolling process. The base metal material 10 can benefit from this effect by containing 0.0005% or more Ca. When the base metal material 10 contains an excessively large amount of calcium, Ca oxide clusters are formed in the steel to cause deterioration in toughness. When the base metal material 10 contains Ca, it is recommended that the Ca content be 0.0050% or less. The Ca content is preferably 0.0040% or less, and more preferably 0.0035% or less. The base metal material 10 preferably contains 0.0008% or more Ca, and more preferably 0.0010% or more Ca. The base metal material 10 preferably contains 0.0008% or more and 0.0040% or less Ca, and more preferably 0.0010% or more and 0.0035% or less Ca.

### B: 0.0050% or less

Boron is an element that contributes to reducing the size of microstructures by lowering the transformation start temperature, and thereby increases the strength of steel. The base metal material 10 can benefit from these effects by containing 0.0002% or more B. When the base metal material 10 contains an excessively large amount of boron, ductility and toughness are lowered. Furthermore, when the base metal material 10 contains an excessively large amount of boron, the hardness of the electric resistance weld 20 may be increased and the corrosion resistance of the heat-affected zones 30 may be lowered. Thus, when the base metal material 10 contains B, it is recommended that the B content be 0.0050% or less. The B content is preferably 0.0005% or more and 0.0040% or less, and more preferably 0.0008% or more and 0.0030% or less.

### Sn: 0.100% or less

Tin is an element that suppresses decarburization stemming from nitridation or oxidation of the steel surface and thereby suppresses a decrease in strength. The base metal material 10 can benefit from these effects by containing 0.001% or more Sn. When the base metal material 10 contains an excessively large amount of tin, ductility and toughness are lowered. Thus, when the base metal material 10 contains Sn, it is recommended that the Sn content be 0.100% or less. The base metal material 10 preferably contains 0.080% or less Sn, and more preferably 0.060% or less Sn. It is recommended that the base metal material 10 contain 0.001% or more Sn. The Sn content is preferably 0.002% or more, and more preferably 0.005% or more.

Here, the Vickers hardness at a position 1 mm deep from the inner surface of the base metal material 10 is defined as the base metal material hardness HB, and the Vickers hardness at a position 1 mm deep from the inner surface of the electric resistance weld 20 is defined as the electric resistance weld hardness HW. It is recommended that the absolute value of the difference between the base metal material hardness HB and the electric resistance weld hardness HW be 100 HV or less, that is, |HW - HB| ≤ 100 HV. The difference in absolute value is preferably 80 HV or less.

When there is a large difference between the base metal material hardness (HB) and the electric resistance weld hardness (HW), local cells are formed due to the difference in material properties between the base metal material 10 and the electric resistance weld 20, and may cause a decrease in the corrosion resistance of the heat-affected zones 30. Sufficient corrosion resistance of the heat-affected zones 30 can be obtained by controlling |HW - HB| to 100 HV or less.

While smaller |HW - HB| is more preferable, excessive reduction leads to an increase in manufacturing costs and an increase in manufacturing loads. It is recommended that |HW - HB| be 2 HV or more. |HW - HB| is preferably 5 HV or more.

The base metal material hardness (HB) and the electric resistance weld hardness (HW) may be measured by a Vickers test. The test may be performed in accordance with the method described in JIS Z 2244 (2020). In the test, the base metal material 10 and the electric resistance weld 20 are both tested with respect to a measurement surface that is a cross section perpendicular to the axial direction of the electric resistance welded steel pipe 100. It is recommended that the load in the test be 1 kgf. For example, the base metal material hardness (HB) and the electric resistance weld hardness (HW) may be determined by measuring the hardness at three sites in a test portion and averaging the values obtained. The measurement portion for the base metal material hardness (HB) may be a portion of the base metal material 10 at a position 90 degrees away from the electric resistance weld 20 in a circumferential direction. The measurement portion for the electric resistance weld hardness (HW) may be the electric resistance weld 20.

It is recommended that the electric resistance welded steel pipe 100 have a yield strength of 400 MPa or more. The yield strength is more preferably 450 MPa or more. When the electric resistance welded steel pipe 100 has a yield strength of 400 MPa or more, sufficient internal pressure resistance can be ensured.

An increase in the yield strength of the electric resistance welded steel pipe 100 may cause a decrease in the corrosion resistance of the electric resistance welded steel pipe 100. Thus, it is recommended that the yield strength be 1100 MPa or less. The yield strength is preferably 1000 MPa or less. The yield strength may be measured by a tensile test. The tensile test is performed in accordance with the provisions in JIS Z 2241. The yield strength (MPa) is the flow stress at a nominal strain of 0.5%. A JIS No. 5 test piece for tensile test is used as the tensile test specimen. The test specimen is sampled from the base metal material 10 so that the tensile direction will be parallel to the axial direction of the electric resistance welded steel pipe 100.

In the electric resistance welded steel pipe 100, it is preferable that the base metal material 10 and the electric resistance weld 20 have a predetermined corrosion rate and a predetermined pitting corrosion growth rate. The corrosion rate and the pitting corrosion growth rate may be measured by the following corrosion test.

Test specimens are sampled from the base metal material 10 and the electric resistance weld 20. The dimensions of the test specimens are 3 mm in thickness × 10 mm in width × 25 mm in length. The width direction of the test specimens is parallel to the circumferential direction of the electric resistance welded steel pipe 100. The longitudinal direction of the test specimens is parallel to the axial direction of the electric resistance welded steel pipe 100. The test specimens are sampled so that the center of their thickness corresponds to a depth of 2.5 mm from the inner surface. The test specimen of the electric resistance weld 20 is sampled from the position at the center of the width.

The test specimens for use in the corrosion test are mirror-polished on all faces and are subsequently degreased with acetone. The corrosion test is performed by exposing the test specimens to an environment containing a mixed gas of SO₂, NO₂, O₂, H₂O, and CO₂ at an increased temperature of 50°C and an increased pressure of 10 MPa. The test time is 72 hours (3 days).

After the test, the test specimens are derusted in accordance with ASTM Standard G1-03, and the corrosion rate is determined. To determine the pitting corrosion growth rate (unit: mm/year), the maximum pitting corrosion depth (unit: mm) on the faces of the test specimen is measured and the value is multiplied by 365/3. The maximum pitting corrosion depth is determined by a microscopic method in accordance with ASTM Standard G46-94.

It is recommended that the corrosion rate measured by the above corrosion test be 0.100 mm/year or less for each of the base metal material 10 and the electric resistance weld 20. Their corrosion rates are preferably 0.090 mm/year or less. It is recommended that the pitting corrosion growth rate measured by the above corrosion test be 0.100 mm/year or less for each of the base metal material 10 and the electric resistance weld 20. Their pitting corrosion growth rates are preferably 0.090 mm/year or less.

Next, a method for manufacturing an electric resistance welded steel pipe according to an embodiment of the present invention will be described. Fig. 2 illustrates a flow in the manufacturing of an electric resistance welded steel pipe. As illustrated in Fig. 2, the method for manufacturing an electric resistance welded steel pipe includes a hot-rolled steel sheet producing step (step S01) of hot-rolling a steel material to produce a hot-rolled steel sheet, and a pipe forming step (step S02) of forming the hot-rolled steel sheet into an open pipe. Furthermore, the method for manufacturing an electric resistance welded steel pipe includes a welding step (step S03) of welding one end portion and the other end portion of the open pipe with each other by electric resistance welding.

The surface temperature of the hot-rolled steel sheet may be measured with, for example, a radiation thermometer.

In step S01, namely, the hot-rolled steel sheet producing step, for example, a steel material having the above-described chemical composition is heated and hot-rolled. Specifically, a steel material containing Cu, Cr, and Mo in a total amount of 0.02 mass% or more is hot-rolled. The steel material that has been hot-rolled is cooled and then coiled into a coil of the hot-rolled steel sheet.

The steel material is also called a steel slab. The steel material may be melted using any known melting technique, such as a converter, an electric arc furnace, or a vacuum melting furnace, without limitation. The steel material may be cast by any known casting method, such as continuous casting, without limitation. The steel material is cast into predetermined dimensions. Instead of continuous casting, an ingot making-blooming method may be adopted. The molten steel may be further subjected to secondary refining, such as ladle refining.

In step S02, namely, the pipe forming step, the steel sheet is formed into a cylindrical shape by, for example, cold roll forming. The open pipe formed in the pipe forming step has a C-shaped cross section perpendicular to the axial direction of the pipe. That is, the open pipe has a gap in the circumferential direction. The gap of the open pipe extends along the axial direction of the pipe.

The heating method for the electric resistance welding performed in step S03, the welding step, may be, for example, Joule heating or induction heating. Step S03, the welding step, is performed in a state that satisfies the following (condition 1) to (condition 3).
(Condition 1) A temperature of 1000°C or above is reached in 1.0 second or less in central regions in the thickness direction (hereinafter, also written as the through-thickness central regions) of portions of the open pipe that are to be welded (hereinafter, also written as the to-be-welded portions).
(Condition 2) The to-be-welded portions have an oxygen concentration of 0.10 mass% or less.
(Condition 3) The amount of molten steel discharge is 0.2 times or more the thickness of the sheet (the sheet thickness) of the open pipe.

For example, condition 1 is achieved by controlling at least one of the pipe-making speed, the heating start position, or the squeeze roll intervals.

When a long time is taken until 1000°C or above is reached in the central regions in the thickness direction of the to-be-welded portions, an increased amount of Cr oxide is formed in the to-be-welded portions. As a result, Cr oxide remains in the electric resistance weld 20 to increase the Cr concentration in the electric resistance weld 20, and the corrosion resistance of the electric resistance weld 20 may be lowered. When a long time is taken until 1000°C or above is reached in the central regions in the thickness direction of the to-be-welded portions, increased amounts of copper and molybdenum are concentrated in the to-be-welded portions. As a result, the concentrations of Cu and Mo in the electric resistance weld 20 are increased, and the corrosion resistance of the heat-affected zones 30 may be lowered. In view of the above, it is recommended that a temperature of 1000°C or above be reached in 1.0 second or less in the central regions in the thickness direction of the to-be-welded portions. The time is preferably 0.8 seconds or less. The temperature of the central regions in the thickness direction of the to-be-welded portions may be measured using a two-color thermometer. For example, the temperature of the central regions in the thickness direction of the to-be-welded portions may be measured with respect to a position that is 20 mm away from a welding start point P1 in the direction opposite to a pipe-making direction D1.

For example, condition 2 is achieved by controlling the composition of the air in the atmosphere in which the to-be-welded portions are placed. Specifically, the oxygen concentration in the atmosphere in which the to-be-welded portions are placed is lowered by spraying nitrogen gas or argon gas to the to-be-welded portions. In this manner, the oxygen concentration in the to-be-welded portions can be lowered. An enclosure may be provided around the to-be-welded portions in order to facilitate controlling the oxygen concentration in the atmosphere. The oxygen concentration in the to-be-welded portions may be calculated from measurement data obtained by measuring the oxygen concentration in the atmosphere with an oxygen concentration meter.

When the oxygen concentration in the to-be-welded portions is high, an increased amount of Cr oxide is formed in the to-be-welded portions. Such Cr oxide will remain in the electric resistance weld. As a result, the concentration of Cr in the electric resistance weld is increased, and the corrosion resistance of the electric resistance weld may be lowered. Furthermore, a high oxygen concentration in the to-be-welded portions leads to an increased amount of Fe oxidation, and thus increases the amounts of copper and molybdenum concentrated in the to-be-welded portions. As a result, the concentrations of Cu and Mo in the electric resistance weld are increased and the corrosion resistance of the heat-affected zones may be lowered. Thus, the oxygen concentration in the to-be-welded portions is 0.10 mass% or less, and preferably 0.08 mass% or less.

Regarding condition 3, the welding power, the pipe-making speed, and the squeeze roll intervals are controlled so that the amount of molten steel discharge will be 0.2 times or more the thickness of the sheet. Fig. 3 illustrates an embodiment of the welding step. As illustrated in Fig. 3, molten steel 13 is formed upon the start of electric resistance welding. The electric resistance welding is performed from the welding start point P1 in the pipe-making direction D1.

The amount of molten steel discharge is expressed as length (mm). Before the to-be-welded portions are continuously photographed with a high-speed camera, the length (mm) per pixel is set beforehand so that the amount of molten steel discharge can be calculated from the length (mm) on the screen. The amount of molten steel discharge is determined by continuously photographing the to-be-welded portions with a high-speed camera. Specifically, the molten steel width W1 is photographed with a high-speed camera for one second at 2000 fps. The 2000 values obtained by photographing are averaged to give the amount of molten steel discharge. For example, a two-dimensional image sensor camera with a high-speed shutter is installed above the welding point, and still images of an area around the welding point are photographed. The photographed images are then binarized to identify the molten steel portions. The amount of molten steel discharge may be determined by calculating the amount corresponding to the molten steel portions.

It is recommended that the molten steel width W1 be measured at a distance L1 from the welding start point P1 toward the downstream in the pipe-making direction. For example, the welding start point P1 may be determined as follows. The butt end faces corresponding to pipe edge portions of the open pipe are detected as a point cloud by image processing. From the point cloud thus detected, two straight lines corresponding to the butt end faces are calculated by the least squares method. The intersection of the calculated two straight lines is determined. This intersection can be taken as the welding start point P1.

The molten steel width W1 may be measured as the distance from the axis AX of the electric resistance welded steel pipe 100 to the base metal material 10. It is recommended that the distance L1 be twice the thickness of the sheet. This location allows the molten steel width W1 to be measured while ensuring that the variation in molten steel width W1 is small and the influence of the welding conditions is appropriately reflected in the molten steel width W1.

When the amount of molten steel discharge is small, Cr oxide is not discharged sufficiently and remains in the electric resistance weld 20, and the corrosion resistance of the electric resistance weld 20 may be lowered. When the amount of molten steel discharge is small, concentrated copper and molybdenum are not discharged sufficiently and remain in the electric resistance weld 20, and the corrosion resistance of the heat-affected zones 30 may be lowered. Thus, it is recommended that the amount of molten steel discharge be 0.2 times or more the thickness of the sheet. The amount of molten steel discharge is preferably 0.3 times or more the thickness of the sheet.

When the amount of molten steel discharge is large, the to-be-welded portions are melted excessively and a sufficient upset cannot be applied. As a result, Cr oxide is not discharged sufficiently and remains in the electric resistance weld 20, and the corrosion resistance of the electric resistance weld 20 may be lowered. Furthermore, concentrated copper and molybdenum are not discharged sufficiently and remain in the electric resistance weld 20, and the corrosion resistance of the heat-affected zones 30 may be lowered. Thus, it is preferable that the amount of molten steel discharge be 3.0 times or less the thickness of the sheet, more preferably 2.0 times or less the thickness of the sheet.

The electric resistance welding may be followed by heat treatment to control the hardness of the electric resistance weld 20. In this case, the whole of the electric resistance welded steel pipe 100 may be heat-treated, or only the electric resistance weld 20 may be heat-treated. For example, the heating method in the heat treatment may be induction heating. However, the method is not limited to such heating, and a heating furnace may be used.

Whether or not the steel pipe qualifies as an electric resistance welded steel pipe can be determined by measuring the width of the electric resistance weld 20 in a cross section cut in the direction perpendicular to the axial direction of the steel pipe. When a cross section of the steel pipe is corroded, for example, the electric resistance weld 20 can be visually recognized as a region that differs in microstructures and contrast from the base metal material 10 and the heat-affected zones 30.

Specifically, an electric resistance welded steel pipe 100 made of carbon steel or low-alloy steel has an electric resistance weld 20 that, when corroded with Nital and observed under an optical microscope, looks whiter than a base metal material 10 and heat-affected zones 30. An example of the electric resistance welded steel pipes 100 made of carbon steel or low-alloy steel is UOE steel pipes. An electric resistance weld 20 of a UOE steel pipe, when corroded with Nital and observed under an optical microscope, shows cellular or dendritic solidified microstructures. It is recommended that the etching solution used to corrode the steel pipes be selected appropriately in accordance with the steel components and the type of steel pipe.

The steel pipe qualifies as an electric resistance welded steel pipe when the electric resistance weld 20 observed as described above has a width in the circumferential direction of the pipe of 1.0 µm or more and 1000 µm or less throughout the thickness of the pipe.

The electric resistance welded steel pipe 100 described above may be used as, for example, a line pipe that constitutes a pipeline connecting one place to another place. When the pipeline is composed of a plurality of line pipes, the electric resistance welded steel pipe 100 described above may be used as at least one of the line pipes to provide increased corrosion resistance at the location where that line pipe(s) is disposed.

### EXAMPLES

The present invention will be described in greater detail below based on Examples. The present invention is not limited to the following Examples.

Molten steels having a chemical composition described in Table 1 were melted and were cast to give slabs as steel materials. The slabs obtained were heated, hot-rolled, cooled, and then coiled into coils. Thus, hot-rolled steel sheets having a thickness of the sheet described in Table 2 (indicated as the sheet thickness in Table 2) (mm) were obtained. Subsequently, the hot-rolled steel sheets were formed into a cylindrical shape by cold roll forming, and were welded by electric resistance welding under conditions described in Table 2. Thus, electric resistance welded steel pipes having an outer diameter (mm) and a wall thickness (mm) described in Table 2 were obtained.

**[Table 1]**

| No. | Chemical composition (mass%) | | | | | | | | | | | | | | | | |
|---|---|---|---|---|---|---|---|---|---|---|---|---|---|---|---|---|---|
| | C | Si | Mn | P | S | Al | N | Nb | V | Ti | Cu | Ni | Cr | Mo | Ca | B | Sn |
| 1 | 0.051 | 0.24 | 1.55 | 0.007 | 0.0004 | 0.024 | 0.0028 | - | 0.035 | 0.021 | 0.13 | - | 0.04 | - | 0.0021 | - | - |
| 2 | 0.032 | 0.36 | 1.93 | 0.024 | 0.0019 | 0.039 | 0.0031 | 0.053 | 0.019 | 0.034 | 0.20 | 0.08 | 0.01 | 0.08 | 0.0017 | - | 0.025 |
| 3 | 0.154 | 0.15 | 1.06 | 0.032 | 0.0022 | 0.036 | 0.0032 | 0.035 | 0.055 | 0.017 | - | - | 0.01 | - | 0.0023 | - | - |
| 4 | 0.044 | 0.06 | 0.89 | 0.019 | 0.0049 | 0.039 | 0.0044 | 0.011 | 0.032 | 0.024 | 0.15 | 0.15 | 0.06 | 0.09 | - | - | - |
| 5 | 0.038 | 0.20 | 1.47 | 0.008 | 0.0041 | 0.024 | 0.0038 | 0.008 | 0.040 | 0.011 | 0.31 | 0.20 | 0.17 | - | 0.0015 | - | - |
| 6 | 0.060 | 0.22 | 1.57 | 0.007 | 0.0005 | 0.028 | 0.0024 | 0.044 | - | 0.021 | 0.29 | - | - | 0.15 | 0.0026 | - | - |
| 7 | 0.055 | 0.19 | 1.34 | 0.023 | 0.0004 | 0.037 | 0.0034 | 0.019 | 0.037 | 0.013 | 0.17 | - | 0.14 | - | - | - | - |
| 8 | 0.067 | 0.11 | 0.98 | 0.005 | 0.0016 | 0.025 | 0.0031 | 0.026 | 0.056 | 0.010 | 0.08 | - | 1.69 | - | 0.0035 | 0.0010 | - |
| 9 | 0.035 | 0.05 | 0.39 | 0.029 | 0.0035 | 0.025 | 0.0038 | 0.009 | - | 0.008 | 1.24 | 0.53 | - | - | - | - | - |
| 10 | 0.184 | 0.03 | 0.46 | 0.023 | 0.0040 | 0.029 | 0.0027 | 0.018 | 0.015 | 0.045 | 0.07 | - | 0.23 | - | 0.0030 | - | - |
| 11 | 0.071 | 0.23 | 1.76 | 0.008 | 0.0019 | 0.031 | 0.0037 | 0.039 | 0.042 | 0.053 | - | - | - | 0.04 | - | - | 0.013 |
| 12 | 0.145 | 0.10 | 1.25 | 0.028 | 0.0015 | 0.021 | 0.0041 | - | - | - | - | - | - | 0.17 | - | - | 0.004 |
| 13 | 0.060 | 0.15 | 1.33 | 0.008 | 0.0023 | 0.026 | 0.0035 | 0.025 | 0.033 | 0.023 | 0.16 | 0.15 | - | - | 0.0022 | - | - |
| 14 | 0.115 | 0.08 | 1.34 | 0.033 | 0.0010 | 0.032 | 0.0025 | 0.078 | - | - | 0.28 | - | 0.03 | - | - | - | - |
| 15 | 0.080 | 0.15 | 1.45 | 0.022 | 0.0014 | 0.050 | 0.0039 | - | 0.077 | - | - | - | 0.35 | 0.11 | - | - | - |
| 16 | 0.067 | 0.19 | 1.82 | 0.021 | 0.0012 | 0.022 | 0.0032 | - | - | 0.077 | 0.14 | - | - | - | - | - | - |
| 17 | 0.092 | 0.22 | 1.74 | 0.013 | 0.0031 | 0.020 | 0.0033 | - | - | - | 0.31 | 1.89 | - | - | - | - | - |
| 18 | 0.035 | 0.37 | 1.82 | 0.018 | 0.0014 | 0.037 | 0.0044 | - | - | - | 0.26 | - | - | - | - | - | 0.096 |
| 19 | 0.051 | 0.14 | 0.52 | 0.020 | 0.0025 | 0.045 | 0.0043 | 0.032 | 0.025 | 0.033 | 0.12 | 0.07 | 0.05 | 0.03 | 0.0018 | 0.0011 | 0.020 |

| | | | | | | | | | | | | | | | | | |
|---|---|---|---|---|---|---|---|---|---|---|---|---|---|---|---|---|---|
| ·The balance in the chemical composition is Fe and incidental impurities. | | | | | | | | | | | | | | | | | |

**[Table 2]**

| No. | Hot-rolled steel sheet | Electric resistance welding | | | | Electric resistance welded steel pipe | |
|---|---|---|---|---|---|---|---|
| | Sheet thickness (mm) | Time to reach 1000°C or above in through-thickness central regions of to-be-welded portions (sec) | Oxygen concentration in to-be-welded portions (mass%) | Amount of molten steel discharge (mm) | Amount of molten steel discharge/sheet thickness | Outer diameter (mm) | Wall thickness (mm) |
| 1 | 19 | 0.4 | 0.08 | 10 | 0.5 | 550 | 19 |
| 2 | 25 | 0.6 | 0.05 | 18 | 0.7 | 600 | 25 |
| 3 | 16 | 0.7 | 0.04 | 22 | 1.4 | 550 | 16 |
| 4 | 19 | 1.2 | 0.05 | 23 | 1.2 | 550 | 19 |
| 5 | 5 | 0.6 | 0.11 | 7 | 1.3 | 100 | 5 |
| 6 | 16 | 0.6 | 0.06 | 53 | 3.3 | 600 | 16 |
| 7 | 20 | 0.7 | 0.06 | 2 | 0.1 | 600 | 20 |
| 8 | 4 | 0.5 | 0.05 | 3 | 0.7 | 100 | 4 |
| 9 | 3 | 0.4 | 0.08 | 4 | 1.2 | 60 | 3 |
| 10 | 16 | 0.8 | 0.07 | 42 | 2.6 | 400 | 16 |
| 11 | 16 | 0.5 | 0.05 | 24 | 1.5 | 400 | 16 |
| 12 | 20 | 0.5 | 0.07 | 18 | 0.9 | 600 | 20 |
| 13 | 20 | 0.7 | 0.09 | 46 | 2.3 | 600 | 20 |
| 14 | 19 | 0.7 | 0.09 | 21 | 1.1 | 600 | 19 |
| 15 | 20 | 0.8 | 0.05 | 40 | 2.0 | 600 | 20 |
| 16 | 22 | 0.6 | 0.08 | 37 | 1.7 | 650 | 22 |
| 17 | 16 | 0.6 | 0.08 | 37 | 2.3 | 550 | 16 |
| 18 | 16 | 0.4 | 0.04 | 40 | 2.5 | 550 | 16 |
| 19 | 25 | 0.6 | 0.05 | 23 | 0.9 | 600 | 25 |

Test specimens were sampled from the electric resistance welded steel pipes and were subjected to element concentration measurement, tensile test, Vickers test, and corrosion test described later.

### [Amount of molten steel discharge]

The amount (mm) of molten steel discharge is determined by continuously photographing the to-be-welded portions with a high-speed camera. Specifically, the length (mm) per pixel is set beforehand, and the length (mm) on the screen is calculated. The molten steel width W1 is photographed with a high-speed camera for one second at 2000 fps. The 2000 values obtained by photographing were averaged to give the amount of molten steel discharge.

The molten steel width W1 was measured at a distance L1 from the welding start point P1 toward the downstream in the pipe-making direction. The welding start point P1 was set as follows. In the images showing the open pipe, the butt end faces corresponding to pipe edge portions were detected as a point cloud by image processing. From the point cloud thus detected, two straight lines corresponding to the butt end faces were calculated by the least squares method. The intersection of the calculated two straight lines was determined. This intersection was taken as the welding start point P1. The molten steel width W1 was measured as the distance from the axis AX of the electric resistance welded steel pipe 100 to the base metal material 10. It is recommended that the distance L1 be twice the thickness of the sheet. The thickness of the sheet used here was the nominal sheet thickness of the hot-rolled sheet.

### [Element concentration measurement]

The concentrations of elements in the base metal material and the electric resistance weld were measured by the EPMA method. The measurement surfaces of the electric resistance weld and the base metal material were cross sections that were perpendicular to the axial direction of the pipe. In the measurement by the EPMA method, the beam diameter was set to 1 µm.

[Cr]_{B}, [Cu]_{B}, and [Mo]_{B} were determined by measuring the respective concentrations with respect to a total of 9 sites that were centered at a position 90 degrees away from the electric resistance weld 20 in a circumferential direction and were located 1 mm deep from the inner surface at 1 µm intervals in the circumferential direction, and averaging the measured values. [Cr]_{W}, [Cu]_{W}, and [Mo]_{w} were determined by measuring the respective concentrations with respect to a total of 9 sites that were centered at the electric resistance weld and were located 1 mm deep from the inner surface at 1 µm intervals in a circumferential direction, and averaging the measured values.

### [Tensile test]

The tensile test was performed in accordance with the provisions in JIS Z 2241. The yield strength (MPa) was the flow stress at a nominal strain of 0.5%. A JIS No. 5 test piece for tensile test was used as the tensile test specimen. The test specimen was sampled from the base metal material so that the tensile direction would be parallel to the axial direction of the electric resistance welded steel pipe.

### [Vickers test]

The Vickers hardness was measured by a Vickers test. The electric resistance weld and the base metal material were both tested with respect to a measurement surface that was a cross section perpendicular to the axial direction of the pipe, at a position 1 mm deep from the inner surface in accordance with the method described in JIS Z 2244 (2020). The load was 1 kgf. For both the electric resistance weld and the base metal material, the hardness was measured at three sites and the results were averaged to give HW or HB.

### [Corrosion test]

Test specimens were sampled from the base metal material and the electric resistance weld. The dimensions of the test specimens were 3 mm in thickness × 10 mm in width × 25 mm in length. The width direction of the test specimens was parallel to the circumferential direction of the electric resistance welded steel pipe. The longitudinal direction of the test specimens was parallel to the axial direction of the electric resistance welded steel pipe. The test specimens were sampled so that the center of their thickness would correspond to a depth of 2.5 mm from the inner surface. The test specimen of the electric resistance weld was sampled so that the electric resistance weld would be located at the center of the width.

The test specimens for use in the corrosion test were mirror-polished on all faces and were subsequently degreased with acetone. The corrosion test was performed by exposing the test specimens to an environment containing a mixed gas of SO₂, NO₂, O₂, H₂O, and CO₂ at an increased temperature of 50°C and an increased pressure of 10 MPa. The test time was 72 hours (3 days). The gas that was used was CO₂ containing, in volume fraction, 50 ppm SO₂, 300 ppm NO₂, 100 ppm O₂, and 600 ppm H₂O.

After the test, the test specimens were derusted in accordance with ASTM Standard G1-03, and the corrosion rate was determined. To determine the pitting corrosion growth rate (unit: mm/year), the maximum pitting corrosion depth (unit: mm) on the faces of the test specimen was measured and the value was multiplied by 365/3. The maximum pitting corrosion depth was determined by a microscopic method in accordance with ASTM Standard G46-94. The results obtained are described in Table 3.

**[Table 3]**

| No. | Element concentrations in base metal material and electric resistance weld | | | | | | | | | | Mechanical properties of electric resistance welded steel pipe | | | | Corrosion resistance of electric resistance welded steel pipe | | | | Remarks |
|---|---|---|---|---|---|---|---|---|---|---|---|---|---|---|---|---|---|---|---|
| | [Cr]_{B} (mass%) | [Mo]_{B} (mass%) | [CU]_{B} (mass%) | [Cr]_{B}+[Mo]_{B}+[CU]_{B} (mass%) | [Cr]w (mass%) | [Mo]w (mass%) | [Cu]w (mass%) | [Cr]_{W}/[Cr]_{B} | [Mo]_{w}/[Mo]_{B} | [Cu]_{W}/[Cu]_{B} | Yield strength (MPa) | H_{B} (HV) | Hw (HV) | \|H_{w}-H_{B}\| (HV) | Corrosion rate in base metal material (mm/year) | Pitting corrosion growth rate in base metal material (mm/year) | Corrosion rate in electric resistance weld (mm/year) | Pitting corrosion growth rate in electric resistance weld (mm/year) | |
| 1 | 0.04 | 0.00 | 0.13 | 0.17 | 0.03 | 0.00 | 0.10 | 0.75 | - | 0.77 | 501 | 205 | 198 | 7 | 0.047 | 0.039 | 0.060 | 0.038 | Inv. Ex. |
| 2 | 0.01 | 0.08 | 0.20 | 0.29 | 0.00 | 0.10 | 0.26 | - | 1.25 | 1.30 | 469 | 176 | 203 | 27 | 0.053 | 0.035 | 0.038 | 0.006 | Inv. Ex. |
| 3 | 0.01 | 0.00 | 0.00 | 0.01 | 0.01 | 0.00 | 0.00 | 1.00 | - | - | 499 | 202 | 205 | 3 | 0.170 | 0.272 | 0.192 | 0.281 | Comp. Ex. |
| 4 | 0.06 | 0.09 | 0.15 | 0.30 | 0.06 | 0.14 | 0.24 | 1.00 | 1.56 | 1.60 | 487 | 185 | 190 | 5 | 0.073 | 0.040 | 0.227 | 0.152 | Comp. Ex. |
| 5 | 0.17 | 0.00 | 0.31 | 0.48 | 0.27 | 0.00 | 0.53 | 1.59 | - | 1.71 | 531 | 229 | 219 | 10 | 0.032 | 0.049 | 0.061 | 0.295 | Comp. Ex. |
| 6 | 0.00 | 0.15 | 0.29 | 0.44 | 0.00 | 0.23 | 0.51 | - | 1.53 | 1.76 | 447 | 163 | 190 | 27 | 0.005 | 0.033 | 0.323 | 0.481 | Comp. Ex. |
| 7 | 0.14 | 0.00 | 0.17 | 0.31 | 0.12 | 0.00 | 0.28 | 0.86 | - | 1.65 | 478 | 200 | 206 | 6 | 0.050 | 0.019 | 0.057 | 0.256 | Comp. Ex. |
| 8 | 1.69 | 0.00 | 0.08 | 1.77 | 2.38 | 0.00 | 0.08 | 1.41 | - | 1.00 | 547 | 199 | 220 | 21 | 0.055 | 0.070 | 0.057 | 0.056 | Inv. Ex. |
| 9 | 0.00 | 0.00 | 1.24 | 1.24 | 0.00 | 0.00 | 1.41 | - | - | 1.14 | 572 | 241 | 183 | 58 | 0.096 | 0.029 | 0.034 | 0.019 | Inv. Ex. |
| 10 | 0.23 | 0.00 | 0.07 | 0.30 | 0.18 | 0.00 | 0.07 | 0.78 | - | 1.00 | 474 | 171 | 183 | 12 | 0.051 | 0.038 | 0.067 | 0.056 | Inv. Ex. |
| 11 | 0.00 | 0.04 | 0.00 | 0.04 | 0.00 | 0.05 | 0.00 | - | 1.25 | - | 452 | 172 | 159 | 13 | 0.066 | 0.010 | 0.027 | 0.063 | Inv. Ex. |
| 12 | 0.00 | 0.17 | 0.00 | 0.17 | 0.00 | 0.24 | 0.00 | - | 1.41 | - | 459 | 164 | 191 | 27 | 0.046 | 0.070 | 0.058 | 0.020 | Inv. Ex. |
| 13 | 0.00 | 0.00 | 0.16 | 0.16 | 0.00 | 0.00 | 0.23 | - | - | 1.44 | 488 | 173 | 187 | 14 | 0.055 | 0.057 | 0.050 | 0.067 | Inv. Ex. |
| 14 | 0.03 | 0.00 | 0.28 | 0.31 | 0.04 | 0.00 | 0.32 | 1.33 | - | 1.14 | 458 | 189 | 149 | 40 | 0.053 | 0.066 | 0.021 | 0.075 | Inv. Ex. |
| 15 | 0.35 | 0.11 | 0.00 | 0.46 | 0.32 | 0.11 | 0.00 | 0.91 | 1.00 | - | 476 | 210 | 161 | 49 | 0.074 | 0.033 | 0.070 | 0.055 | Inv. Ex. |
| 16 | 0.00 | 0.00 | 0.14 | 0.14 | 0.00 | 0.00 | 0.19 | - | - | 1.36 | 453 | 179 | 229 | 50 | 0.075 | 0.050 | 0.029 | 0.069 | Inv. Ex. |
| 17 | 0.00 | 0.00 | 0.31 | 0.31 | 0.00 | 0.00 | 0.27 | - | - | 0.87 | 488 | 201 | 176 | 25 | 0.044 | 0.014 | 0.046 | 0.040 | Inv. Ex. |
| 18 | 0.00 | 0.00 | 0.26 | 0.26 | 0.00 | 0.00 | 0.29 | - | - | 1.12 | 425 | 171 | 141 | 30 | 0.063 | 0.073 | 0.006 | 0.085 | Inv. Ex. |
| 19 | 0.05 | 0.03 | 0.12 | 0.20 | 0.06 | 0.02 | 0.13 | 1.20 | 0.67 | 1.08 | 580 | 220 | 237 | 17 | 0.087 | 0.055 | 0.079 | 0.076 | Inv. Ex. |

In Table 3, the electric resistance welded steel pipes Nos. 1, 2, 8, 9, and 10 to 19 represent Inventive Examples, and the electric resistance welded steel pipes Nos. 3, 4, 5, 6, and 7 represent Comparative Examples.

All of the electric resistance welded steel pipes of Inventive Examples satisfy [Cr]_{B} + [Mo]_{B} + [Cu]_{B} ≥ 0.02; when [Cr]_{B} ≥ 0.20, [Cr]_{W}/[Cr]_{B} ≤ 1.50; when [Mo]_{B} ≥ 0.20, [Mo]_{W}/[Mo]_{B} ≤ 1.50; and when [Cu]_{B} ≥ 0.20, [Cu]_{w}/[Cu]_{B} ≤ 1.50.

The electric resistance welded steel pipe No. 3 of Comparative Example failed to attain the desired corrosion resistance because [Cr]_{B} + [Mo]_{B} + [Cu]_{B} was below the range of the present invention.

In the electric resistance welded steel pipe No. 4 of Comparative Example, a long time was taken until the central regions in the thickness direction of the to-be-welded portions reached 1000°C or above during the electric resistance welding, and consequently [Mo]_{w}/[Mo]_{B} and [Cu]_{W}/[Cu]_{B} exceeded 1.50. As a result, the desired corrosion resistance was not obtained.

In the electric resistance welded steel pipe No. 5 of Comparative Example, the oxygen concentration in the to-be-welded portions during the electric resistance welding was high, and consequently [Cr]_{W}/[Cr]_{B} and [Cu]_{W}/[Cu]_{B} exceeded 1.50. As a result, the desired corrosion resistance was not obtained.

In the electric resistance welded steel pipe No. 6 of Comparative Example, the amount of molten steel discharge during the electric resistance welding was large, and consequently [Mo]_{w}/[Mo]_{B} and [Cu]_{W}/[Cu]_{B} exceeded 1.50. As a result, the desired corrosion resistance was not obtained.

In the electric resistance welded steel pipe No. 7 of Comparative Example, the amount of molten steel discharge during the electric resistance welding was small, and consequently [Cu]_{W}/[Cu]_{B} exceeded 1.50. As a result, the desired corrosion resistance was not obtained.

### Reference Signs List

- 100: electric resistance welded steel pipe
- 10: base metal material
- 20: electric resistance weld
- 30: heat-affected zone

## Claims

1. An electric resistance welded steel pipe comprising a base metal material, and an electric resistance weld connecting one end portion of the base metal material and other end portion of the base metal material to each other,
wherein
the base metal material and the electric resistance weld contain at least one of Cr, Cu, or Mo, and
relationships between concentrations of Cr, Cu, and Mo in the base metal material and concentrations of Cr, Cu, and Mo in the electric resistance weld satisfy the following expression: ${\left[Cr\right]}_{B} + {\left[Cu\right]}_{B} + {\left[Mo\right]}_{B} \geq 0.02$
and further satisfy expression (1) when the base metal material contains 0.02 mass% or more Cr; satisfy expression (2) when the base metal material contains 0.02 mass% or more Cu; and satisfy expression (3) when the base metal material contains 0.02 mass% or more Mo, ${\left[Cr\right]}_{W} / {\left[Cr\right]}_{B} \leq 1.50$ ${\left[Cu\right]}_{W} / {\left[Cu\right]}_{B} \leq 1.50$ ${\left[Mo\right]}_{W} / {\left[Mo\right]}_{B} \leq 1.50$
wherein [Cr]_{B} is the concentration (mass%) of Cr in the base metal material, [Cr]_{W} is the concentration (mass%) of Cr in the electric resistance weld, [Cu]_{B} is the concentration (mass%) of Cu in the base metal material, [Cu]_{W} is the concentration (mass%) of Cu in the electric resistance weld, [Mo]_{B} is the concentration (mass%) of Mo in the base metal material, and [Mo]_{w} is the concentration (mass%) of Mo in the electric resistance weld.

2. The electric resistance welded steel pipe according to claim 1, wherein the base metal material has a chemical composition comprising, in mass%:
C: 0.020% or more and 0.200% or less,
Si: 0.50% or less,
Mn: 0.50% or more and 2.00% or less,
P: 0.050% or less,
S: 0.0200% or less,
Al: 0.005% or more and 0.100% or less, and
N: 0.0100% or less,
and further comprising at least one of:
Cr: 5.00% or less,
Cu: 2.00% or less, or
Mo: 2.00% or less,
the balance being Fe and incidental impurities.

3. The electric resistance welded steel pipe according to claim 2, wherein the chemical composition of the base metal material further comprises, in mass%, at least one selected from:
Nb: 0.080% or less,
V: 0.080% or less,
Ti: 0.080% or less,
Ni: 2.00% or less,
Ca: 0.0050% or less,
B: 0.0050% or less, and
Sn: 0.100% or less.

4. The electric resistance welded steel pipe according to any one of claims 1 to 3, which has a difference in Vickers hardness of 100 HV or less in absolute value between the Vickers hardness at a position 1 mm deep from an inner surface of the electric resistance weld and the Vickers hardness at a position 1 mm deep from an inner surface of the base metal material.

5. A line pipe using the electric resistance welded steel pipe described in any one of claims 1 to 4.

6. A method for manufacturing an electric resistance welded steel pipe comprising a hot-rolled steel sheet producing step of heating and hot-rolling a steel material to produce a hot-rolled steel sheet; a pipe forming step of forming the hot-rolled steel sheet into an open pipe; and a welding step of welding one end portion and other end portion of the open pipe with each other by electric resistance welding, wherein
the steel material that is heated and hot-rolled to produce a hot-rolled steel sheet in the hot-rolled steel sheet producing step contains Cu, Cr, and Mo in a total amount of 0.02 mass% or more, and
the welding step is performed under conditions where a temperature of 1000°C or above is reached in 1.0 second or less in central regions in a thickness direction of portions of the open pipe that are to be welded, the portions of the open pipe that are to be welded have an oxygen concentration of 0.10 mass% or less, and an amount of molten steel discharge is 0.2 times or more a sheet thickness of the open pipe.
